

May 2, 1961

M. M. SHIHADEH

2,982,396

PACKAGING UNIT AND PROCESS FOR MAKING SAME

Filed Jan. 29, 1960



Fig. 1



Fig. 2

MUSA M. SHIHADEH

INVENTOR.

BY

*Karl F. Porr*  
AGENT

1

2,982,396

## PACKAGING UNIT AND PROCESS FOR MAKING SAME

Musa M. Shihadeh, 267 Dean St., Brooklyn 17, N.Y.

Filed Jan. 29, 1960, Ser. No. 5,539

24 Claims. (Cl. 206—47)

My present invention relates to a single-container packaging unit for a plurality of chemically reactive components, and to a process for making such units.

Multi-component chemical systems and, more particularly, systems wherein at least two components (e.g. polymerizable compounds and their activators) are adapted to interact upon suitable agitation to obtain a desired end product, have hitherto required the individual packaging of each reactive component or, with joint storage, the physical separation of the components by means of a removable barrier to avoid premature formation of the end product.

It is an object of the present invention to provide a one-package unit with two or more chemically reactive components which is adapted to effect savings in material costs and to enable simplified processing by the elimination of separate packaging for individual components.

It is another object of the invention to provide a packaging system for jointly storing a plurality of reactive components for relatively long periods without detriment.

It is still another object of my invention to provide a packaging system for two or more components, adapted to be combined prior to use, wherein the disadvantages of handling a plurality of containers are obviated.

According to a feature of the invention, a miscible barrier layer not requiring subsequent removal is interposed between masses of chemically reactive materials in a single container. The barrier is designed to be relatively inert to attack by either reactive constituent adjacent thereto and to be impermeable by same while, however, being chemically compatible with the mixture resulting from the combination of the components between which it is sandwiched. I have found that this interposed layer may advantageously comprise an ingredient adapted to impart desirable properties to the mixture. The barrier thus may be essentially constituted of, for example, pigmentitious matter adapted to color the mixture, a refractory material designed to enhance fire-retarding properties, a viscosity modifier, a drying inhibitor or accelerator, or a substance capable of modifying the structural strength of the mixture or imparting thixotropic properties thereto.

I have found further that a substantially inert and impermeable barrier of the character described, adapted to resist the diffusion of either reactive component into the other for relatively long periods while permitting the entire contents of the one-package system including the barrier to be stirred into a substantially homogeneous and compatible mixture, may include as its major constituent one or more of the following: drying and non-drying oils, varnishes, alkyds and derivatives thereof, waxes, gels, petroleum and coal-tar derivatives, as well as glycols, polyols, fatty acids and their derivatives. This barrier may be interposed between a wide variety of reactive compounds, including, on the one hand, polymerizable and cross-linking polyfunctional organic substances such as unpolymerized or partially polymerized epoxy resins, polyure-

2

thanes and polyisocyanates, polyalkylene polysulfides, chlorosulfonated polyethylenes, vulcanizable elastomers and halogenated derivatives thereof, and unsaturated polyesters; and, on the other hand, the activators, catalysts, 5 vulcanizers and driers for these substances.

According to another feature of the invention the container is initially charged with one reactive component and subsequently with the barrier composition which forms a layer above the previously introduced reactive component. The other reactive component, adapted to combine chemically with the first one upon the agitation of the 10 contents of the container, is then deposited upon the barrier layer which physically separates the two components. To diminish the risk of intermixing the reactive components 15 when charging the container, the less dense reactive component (generally the activator or catalyst) is preferably deposited on the barrier layer while the denser reactive component (generally the polymerizable substance or base) is positioned therebelow, particularly if the barrier 20 composition is a liquid. It then advantageously should be selected to have a viscosity and a density intermediate those of the reactive components between which it is sandwiched. Alternatively the barrier layer may be of a 25 thixotropic nature, partially solidifying upon introduction to the container, or a substance which has a relatively low melting point and is, therefore, solid at the storing ambient temperature. Since the reaction between components is generally exothermic, the temperature of the 30 contents of the container may be raised sufficiently above the melting point of the barrier layer upon the introduction, for example, of the mixing paddle into the batch. The layer, thus raised above the melting point and in a liquid state, may then be stirred into the component mixture as previously mentioned. Moreover, the barrier 35 layer may also be a super-cooled liquid or a gel. Similarly, the frictional heat of mixing may be sufficient to liquefy the layer.

The invention is further illustrated, but not limited, by the following examples, wherein the parts referred to are on a weight basis. The examples will be more readily understood with reference to the accompanying drawing, in which Figs. 1 and 2 show one-container packaging systems according to the invention with two and three components respectively.

45 More particularly, Fig. 1 shows a container 10 charged with an upper component A of low density, a lower component B of high density and an intervening barrier layer.

## Example 1

|                 | Component A:                | Parts |
|-----------------|-----------------------------|-------|
|                 | Activator (polyamide resin) | 70    |
| Barrier C:      |                             |       |
|                 | Non-drying alkyd            | 20    |
|                 | Carbon black                | 7     |
| 55 Component B: |                             |       |
|                 | Epoxy resin                 | 100   |
|                 | Silica                      | 70    |
|                 | Barytes                     | 50    |

60 Component B, comprising a liquid epoxy resin formed by any diepoxy reaction between a polyhydroxy compound and either epichlorohydrin or dichlorohydrin, is formed by mixing the epoxy resin with commercially available silica and baryte extenders in the proportions shown. A suitable epoxy resin having an epoxide equivalent of 175 to 290 (molecular weight per epoxy group), an average molecular weight of 340 to 450, and a viscosity of 500 to 3500 cps. is manufactured by the Shell Chemical Company under the trade name "Epon." The 65 extenders, having particle sizes ranging between 40 and 325 mesh, are uniformly dispersed throughout the liquid epoxy resin. The component B is introduced into the container 70

tainer 10, shown in the figure, forming a mass upon which the barrier C is deposited.

The barrier C comprises a non-drying alkyd of the type marketed under the name "Paraplex G-20" by Rohm and Haas Co. The alkyd is 100% unmodified and has an acid number of 10 to 20, weighing between 0.97 and 1.1 kg. per liter. A pigmentitious material such as carbon black is dispersed in a heated portion of the alkyd and ground to a fineness of approximately 5 to 6 on the Hegeman scale. Atop the barrier C I deposit a polyamide resin adapted to polymerize the epoxy resin of component B when the contents of the container are mixed. The polyamide resin, forming component A, advantageously has an amine value ranging between 210 and 320 (milligrams of potassium hydroxide equivalent to the base content of 1 gm. of polyamide, as determined by titration with HCl) and a viscosity ranging between 2,000 to 6,000 cps. at a temperature of 20° to 100° C. A suitable polyamide resin is available from General Mills Inc. under the name "Versamide."

The container 10, holding 69% by weight of component B, 9.5% of barrier C and 21.5% of component A, is then closed. The packaging system is found to be stable at room temperatures for a period of greater than 12 months, under normal storage, and for a relatively long period under conditions of severe handling and elevated temperature.

#### Example II

Components A and B:

As in Example I

Barrier C:

Coal-tar derivative \_\_\_\_\_ parts 20  
Titanium dioxide \_\_\_\_\_ do 7

A barrier layer comprising a polymeric coal-tar derivative is interposed between the previously described components A and B. The barrier C, advantageously containing a titanium-dioxide pigment of the type marketed under the name "Titanox Ranc" dispersed in the coal-tar derivative, is treated as described with reference to Example I. A suitable coal-tar derivative is the mixture of polynuclear aromatic hydrocarbons having a melting point less than 5° C., a flash point between 140° and 175° C., a viscosity in the range of from 295 to 4000 cps. at 25° C., and a specific gravity of 1.05, available under the name "Transphalt" from the Pennsylvania Industrial Chemical Corp.

#### Example III

Components A and B:

As in Example I

Barrier C:

Chlorinated wax \_\_\_\_\_ parts 20  
Pigment \_\_\_\_\_ do 3 to 7

A barrier comprising chlorinated paraffin compounds and a pigment (either carbon black or titanium dioxide) is used in place of the barriers previously described in Examples I and II. The chlorinated paraffin compounds, having a chlorine content ranging between 40% and 72% an average molecular weight between 570 and 1060 and a melting point below 95° C., have a viscosity ranging from 20 poises to solid at normal room temperature. Some of these compounds must be heated above their melting points to permit the barrier composition to be poured into the container. Since the barrier will be substantially solid at room temperature, it will possess great mechanical strength prior to stirring and render the packaging system stable for long periods. The heat evolved in the exothermic reaction between components A and B is generally sufficient to melt the barrier and to permit the mixing of the contents into a homogeneous mass.

#### Example IV

Components A and B:

As in Example I

Barrier C:

Chlorinated polyphenyls \_\_\_\_\_ 20 parts.  
Pigments \_\_\_\_\_ as required.

In the present example, the components A and B of Example I are separated by a barrier comprising one or more of the chlorinated polyphenyls (e.g. biphenyls and terphenyls) ranging in viscosity from a mobile liquid to a sticky resin having a softening point below 75° C. (from 35 to 850 saybols at about 52° C.), a density of 1.182 to 1.650 at 25° C., and ranging from 54% to 68% of chlorination.

#### Example V

Components A and B:

As in Example I

Barrier C:

Terpene polymers \_\_\_\_\_ 20 parts.  
Pigments \_\_\_\_\_ as required.

I have found that terpene polymers and mixtures thereof, having a melting range from 10° to 70° C., are also satisfactory barriers between components A and B of Example I. Terpene polymers having molecular weights below 1100, acid numbers less than 4 and saponification numbers less than 4 are available from the Pennsylvania Industrial Chemical Company under the name "Piccolyte."

#### Example VI

Components A and B:

As in Example I

Barrier C:

Petrolatum \_\_\_\_\_ 20 parts.  
Pigments \_\_\_\_\_ as required.

The barrier between the components A and B includes as a major constituent, petrolatum, a semi-solid fraction of the petroleum refining process at storage temperatures. The petrolatum, commonly referred to as petroleum jelly, requires heating and melting to facilitate its application.

#### Example VII

Components A and B:

As in Example I

Barrier C:

Chlorinated wax \_\_\_\_\_ 10 parts.  
Microcrystalline wax \_\_\_\_\_ 10 parts.  
Pigments \_\_\_\_\_ as required.

Microcrystalline wax, a product extracted from refinery still residues and comprising molecules having approximately 41 to 50 carbon atoms, has a melting range from 55° to 75° C. The microcrystalline wax is mixed with chlorinated wax (previously described) and pigment in the proportions shown at a temperature sufficiently high to liquefy both major components (e.g. 80° C.). The liquid barrier mixture is divided into two portions, one of which is poured over the component B previously introduced into the container. The composition is permitted to cool and solidify, whereupon the second portion is poured onto the solidified surface to fill any gaps therein and to seal completely the component B from any contact with the activator (component A) which is poured onto the now solidified barrier. There is no danger, therefore, that cracks or gaps in a solid barrier layer will permit even a trickle of activator to percolate through and contact the epoxy base in component B. A similar technique may be used, if necessary, wherever the barrier comprises a substance which is a solid or semi-solid at storage temperatures.

#### Example VIII

Components A and B:

As in Example I

Barrier C:

30% solution of cellulose acetobutyrate \_\_\_\_\_ 30 parts.  
½ sec. \_\_\_\_\_  
Pigments \_\_\_\_\_ as required.

75 A 30% solution of cellulose acetobutyrate ½ sec. in

Components A and B:

As in Example I

acetate ester has also been found to be an effective barrier in combination with pigmentous material, or in the absence thereof, between the components A and B.

*Example X*

|                                          | Parts |
|------------------------------------------|-------|
| Component A:                             |       |
| Ricinoleyl alcohol                       | 35    |
| Whiting                                  | 100   |
| Tributyl phosphate                       | 30    |
| Colloidal silica                         | 10    |
| Barrier C:                               |       |
| Epoxy ester                              | 30    |
| Whiting                                  | 50    |
| Component B:                             |       |
| Prepolymer of urethane                   | 100   |
| Whiting                                  | 50    |
| Colloidal silica                         | 15    |
| Plasticizer (e.g. chlorinated biphenyls) | 20    |

Component B comprises as a major constituent prepolymers of urethane (e.g. "Solithin 113" of the Thiokol Chemical Co.) having isocyanate reactive terminals and adapted to form a curable polymer with the major active constituent of component A, ricinoleyl alcohol. Whiting and silica serve as extender fillers and pigments, and are ground in vehicles such as tributyl phosphate (component A), the plasticizer (component B) and the barrier substance. The barrier, interposed between the two components as previously described as, for instance, in Example I, comprises a compound resulting from epoxy esterification reactions and present in xylol solution. A suitable solution having 70% solids (epoxy ester) is marketed by Jones-Dabney and Co. under the name "Epi-Tex 1311."

*Example IX*

|                                       | Parts |
|---------------------------------------|-------|
| Component A:                          |       |
| Ricinus oil                           | 100   |
| Whiting                               | 100   |
| Colloidal silica                      | 10    |
| Barrier C:                            |       |
| "Piccopale" resin                     | 20    |
| Whiting                               | 50    |
| Component B:                          |       |
| Polyisocyanate                        | 100   |
| Whiting                               | 50    |
| Colloidal silica                      | 15    |
| Plasticizer (e.g. tributyl phosphate) | 20    |

"Piccopale" is a hydrocarbon resin produced by the polymerization of unsaturated compounds resulting from a petroleum-refining process, having a softening point between 65° and 90° C. The barrier of this example is formed by grinding the pigment (whiting) in the warmed resin. The barrier may be added to the container as described in Example VII, to separate the polyisocyanate from the ricinus oil (castor oil) adapted to react therewith.

Similarly, the barrier of Example X may comprise halogenated (e.g. chlorinated) wax, halogenated polyphenyls, terpene polymers, non-drying alkyds and coal-tar derivatives, all previously described.

*Example XI*

|                             | Parts |
|-----------------------------|-------|
| Component A:                |       |
| Lead dioxide                | 7.5   |
| Dibutyl phthalate           | 6     |
| Stearic acid (inhibitor)    | 1     |
| Barrier C:                  |       |
| Chlorinated biphenyls       | 10    |
| Chlorinated wax             | 10    |
| Triple-pressed stearic acid | 3     |
| Component B:                |       |
| Polyalkylene polysulfide    | 100   |
| Whiting                     | 30    |
| Carbon black                | 3     |
| Titanium dioxide            | 10    |

An organic polysulfide base such as a polyalkylene

polysulfide adapted to form a rubber-like material (e.g. "Thiokol LP-32" of the Thiokol Chemical Corp.) is compounded with pigments in the proportions shown and introduced into the container. A barrier composition is added by the two-step process described in Example VII. The lead-dioxide activator in dibutyl phthalate plasticizer is then added to the container above the hardened barrier layer. The latter, comprising chlorinated waxes (e.g. of the type marketed under the name "Chlorowax") and biphenyls (e.g. "Arochlor"), acts in addition as the carrier for the retarding agent, stearic acid, adapted to slow the rate of reaction when the contents of the container are agitated. A semi-solid, pasty barrier may be formed by the inclusion of petrolatum in the barrier composition, thereby permitting the barrier to be poured without heating. Other compounds which may be incorporated in a barrier composition between the polyalkylene polysulfide and its activator include polyisobutylene, Piccopale resin, epoxy ester, and terpene polymers.

In some instances it will be desirable to arrange the components according to viscosity rather than density. This will be true with two-component systems as well as with multi-component systems incorporating two or more barriers. An example of such multi-component chemical system, comprising three reactive components and two barrier layers therebetween as shown in Fig. 2, is given below.

*Example XII*

|                          | Parts |
|--------------------------|-------|
| Component A':            |       |
| Tertiary amine           | 40    |
| Barrier C':              |       |
| Chlorinated biphenyls    | 20    |
| Component A'':           |       |
| Polyalkylene polysulfide | 130   |
| Colloidal silica         | 20    |
| Calcium carbonate        | 50    |
| Barrier C'':             |       |
| Chlorinated wax          | 20    |
| Component B:             |       |
| Epoxy resin              | 130   |
| Colloidal silica         | 20    |
| Calcium carbonate        | 50    |

Component B, comprising an intimate mixture of a liquid epoxy resin, as described in Example I, with colloidal silica and calcium carbonate, which serve as pigments and extenders, is introduced into the container as the first, most viscous component. A barrier layer C'' of chlorinated wax, having a viscosity ranging from 20 poises to solid at normal room temperature, is then deposited on top of component B, to receive the second reactive component A''. Polyalkylene polysulfides, including one or more of the polymers produced by the chemical reaction between dichlorodiethylformal and an alkali polysulfide, as liquid polymers, water-dispersed latices and emulsions, organic polysulfide rubbers and related forms, and particularly the Thiokol products marketed under the designations LP-2, LP-32, LP-3, LP-33 and LP-8, are admixed with colloidal silica and calcium carbonate to form a layer of component A'' on top of barrier C''. "Thiokol" LP-32, typical of the liquid polymers, has a specific gravity of 1.27 at 20° C., an average molecular weight of 4000, an open-cup flash point of approximately 230° C. and a viscosity of 350 to 450 poises at 25° C. A second barrier C', comprising chlorinated biphenyls of the type marketed under the trade name of "Arochlor" 1254, 1258, 1260 and 1262 and having respective chlorine contents of 54%, 58%, 60% and 62%, is deposited above the layer of component A''. These chlorinated biphenyls have been described in Example IV. The final reactive component A', to be introduced into the one-package system above the barrier C', comprises a tertiary-amine activator for the components A'' and B. Component A' may include a substituted aminomethylphenol of the type marketed under the name "DMP 10" by Rohm and Haas Co.

Since the barrier composition is selected to impart desired properties to the finished mix (e.g. as in Example I wherein it acts as a plasticizer, fire-retarder and low-cost filler), it will be apparent that the compositions may be altered, proportions changed and compounds interchanged or added as required for a particular purpose. The invention may readily be seen to extend to many reaction systems, not described, known to persons skilled in the art and intended to be included within the spirit and scope of the invention except as further limited by the appended claims.

I claim:

1. A packaging unit comprising a container, a first and a second component in said container capable of interacting with each other, and a barrier layer separating said components, said layer consisting at least in part of a material foreign to said components but compatible with their interaction product.

2. A unit according to claim 1 wherein said layer is solid.

3. A unit according to claim 2 wherein said layer consists to a major extent of wax.

4. A unit according to claim 1 wherein said layer contains a colorant for said interaction product.

5. A unit according to claim 1 wherein said layer contains a fire-retarding agent for said interaction product.

6. A packaging unit comprising a container, a lower and an upper component in said container capable of interacting with each other, and a horizontal barrier layer separating said components, said layer consisting at least in part of a material foreign to said components but compatible with their interaction product.

7. A unit according to claim 6 wherein said lower component has a density greater than that of said upper component.

8. A unit according to claim 7 wherein said barrier layer is a liquid having a density intermediate the densities of said components.

9. A unit according to claim 8 wherein a major proportion of said barrier layer consists of a non-drying alkyd.

10. A unit according to claim 6 wherein said layer contains a thixotropic substance as a major ingredient.

11. A unit according to claim 10 wherein said thixotropic substance is petroleum jelly.

12. A packaging unit comprising a container, a first and a second component in said container capable of combining with each other in an exothermic reaction, and a substantially solid barrier layer separating said components, said layer being liquefiable by the exothermic reaction and compatible with the reaction product formed thereby.

13. A unit according to claim 12 wherein said layer consists to a major extent of a mixture of microcrystalline and halogenated waxes.

14. A packaging unit comprising a container, a polymerizable organic compound in said container, a polymerization promoter in said container, and a barrier layer separating said compound from said promoter, said barrier layer consisting of a material compatible with the polymerized compound.

15. A unit according to claim 14 wherein said barrier layer contains a polymerization-retarding agent.

16. A process for packaging two components capable of interacting with each other, comprising the steps of introducing one of said components into a container, topping said one component with a barrier layer of a material compatible with the interaction product of said components, depositing on said layer the other of said

components, storing the container so charged, and subsequently initiating interaction of said components by stirring the contents of said container into a mixture.

5 17. A process according to claim 16 wherein the container is held closed during storage.

18. A process for packaging two components of different densities capable of interacting with each other, comprising the steps of introducing the denser one of said components into a container, topping said denser component with a barrier layer of a material compatible with the interaction product of said components, depositing on said layer the other of said components, storing the container so charged, and subsequently initiating interaction of said components by stirring the contents of said container into a mixture.

19. A process for packaging two components capable of exothermally interacting with each other, comprising the steps of introducing one of said components into a container, liquefying a barrier material which is substantially solid at ambient temperatures and compatible with

20 the interaction product of said components, introducing the so liquefied material into the container as a separating layer overlying said one component, allowing said layer to solidify, depositing on the so solidified layer the other of said components, storing the container so charged, subsequently heating the container sufficiently to liquefy said layer, and initiating interaction of said components by stirring the contents of said container into a mixture.

25 20. A process according to claim 19 wherein said barrier material is introduced into the container in stages, a part of the liquefied material being added after solidification of a previously deposited portion.

21. A process for packaging two components of different viscosities capable of interacting with each other, comprising the steps of introducing the more viscous one of said components into a container, topping said more viscous component with a barrier layer of a material compatible with the interaction product of said components, depositing on said layer the other of said components, storing the container so charged, and subsequently initiating interaction of said components by stirring the contents of said container into a mixture.

22. A packaging unit comprising a container, three components in said container capable of interacting with each other, a barrier layer separating one of said components from a second of said components, and another barrier layer separating the third component from said second of said components.

23. A packaging unit comprising a container, a first component consisting in major part of a polyalkylene polysulfide, a second component consisting in major part of a compound adapted to react with and cure said polyalkylene polysulfide in said container, and a barrier layer separating said components, said layer consisting at least in part of a material foreign to said components but compatible with their interaction products.

24. A packaging unit comprising a container, a first component consisting in major part of an epoxy resin, a second component consisting in major part of a compound adapted to react with and cure said epoxy resin in said container, and a barrier layer separating said components, said layer consisting at least in part of a material foreign to said components but compatible with their interaction products.

#### References Cited in the file of this patent

UNITED STATES PATENTS

1,846,052 Grant Feb. 23, 1932